

April 3, 1973

KEISUKE SHIBA ET AL

3,725,074

FOGGED, DIRECT POSITIVE SILVER HALIDE EMULSIONS CONTAINING  
HYDROXYPHTHALEIN DYES AND SULFONATED COMPOUNDS

Filed March 19, 1971

FIG. 1



FIG. 2



INVENTORS

KEISUKE SHIBA

MASANAO HINATA

KOUTARO YAMASUE

TOKIHARU KONDO

BY Sughrue, Rothwell, Mion,  
Zinn & Macpeak  
ATTORNEYS

# United States Patent Office

3,725,074  
Patented Apr. 3, 1973

1

3,725,074  
FOGGED, DIRECT POSITIVE SILVER HALIDE  
EMULSIONS CONTAINING HYDROXYPHTHALEIN DYES AND SULFONATED COMPOUNDS

Keisuke Shiba, Masanao Hinata, Koutaro Yamasue, and  
Tokiharu Kondo, Kanagawa, Japan, assignors to Fuji  
Photo Film Co., Ltd., Kanagawa, Japan

Filed Mar. 19, 1971, Ser. No. 125,992  
Claims priority, application Japan, Mar. 19, 1970,  
45/23,343

Int. Cl. G03c 1/08

U.S. Cl. 96—122

14 Claims

### ABSTRACT OF THE DISCLOSURE

A direct positive silver halide photographic emulsion containing at least one dye represented by the general formula:

(I)



wherein  $X_1$ ,  $X_2$ ,  $X_3$ ,  $X_4$  and  $X_5$  each represents a halogen atom;  $m$ ,  $n$ ,  $L$ , and  $p$  represent 0 or 1;  $q$  represents 0, 1, 2, 3 or 4; providing that when said  $m$ ,  $n$ ,  $L$ ,  $p$  and  $q$  are 0, said  $X_1$ ,  $X_2$ ,  $X_3$ ,  $X_4$  and  $X_5$  each represents a hydrogen atom; and  $M$  represents a member selected from the group consisting of a hydrogen atom, an alkali metal atom,  $\text{NH}_4^+$ , and an alkaline earth metal; together with at least one compound represented by the general formula:

(II)



wherein  $Y$  represents a member selected from the group consisting of  $=\text{CH}-$  and  $=\text{N}-$ ;  $R_1$ ,  $R_2$ ,  $R_3$ , and  $R_4$  each represents a member selected from the group consisting of a hydrogen atom, a hydroxyl group, an alkoxy group, an aryloxy group, a halogen atom, a heterocyclic nucleus, an alkylthio group, a heterocyclithio group, an arylthio group, an amino group, an alkylamino group, a substituted alkylamino group, an arylamino group, a substituted arylamino group, a heterocyclamino group, an aryl group and a mercapto group; and  $-A-$  represents at least one member defined as  $A_1$  and  $A_2$ , said  $A_1$  being a member selected from the group consisting of:

2

wherein  $M$  represents a member selected from the group consisting of a hydrogen atom and a cation giving water solubility to said compound; and said  $A_2$  being a member selected from the group consisting of:

5



10

15

20

30

35

45

50

55

providing that when  $A$  is  $A_2$ , at least one of said  $R_1$ ,  $R_2$ ,  $R_3$  and  $R_4$  is a substituent containing  $-\text{SO}_3\text{M}$ , wherein  $M$  is the same as defined above; and a silver halide photographic emulsion.

### BACKGROUND OF THE INVENTION

#### (1) Field of the invention

This invention relates to a silver halide photographic emulsion and more particularly to a direct positive silver halide photographic emulsion.

#### (2) Description of prior art

It is known that by incorporating a sensitizing dye in a silver halide photographic emulsion which has been preliminarily fogged and capable of directly providing a positive image by exposure and development, the silver halide is spectrally sensitized. It is also known that, depending upon the kind of sensitizing dye employed and the amount of the sensitizing dye added to the emulsion, the contrast of the image obtained is varied.

In general, although by incorporating a sensitizing dye in a direct positive silver halide photographic emulsion the sensitivity thereof increases, it frequently happens that the maximum density ( $D_{\max}$ ) is reduced and the contrast lowered, thus preventing sufficient images from being obtained.

As a result of various studies, we have discovered that a halogen-substituted hydroxyphthalein dye represented by the following general Formula I is an excellent dye for maintaining the definite maximum density and definite contrast and increasing the sensitivity.



## General Formula I:



wherein  $X_1$ ,  $X_2$ ,  $X_3$ ,  $X_4$ , and  $X_5$  each represents a halogen atom;  $M$  represents a hydrogen atom, an alkali metal (such as Na or K),  $NH_4$ , or an alkaline earth metal (such as  $\frac{1}{2}Ca$ );  $m$ ,  $n$ ,  $L$ , and  $p$  represent 0 or 1;  $q$  represents 0, 1, 2, 3, or 4; said  $X_1$ ,  $X_2$ ,  $X_3$ ,  $X_4$ , and  $X_5$  being a hydrogen atom when  $m$ ,  $n$ ,  $L$ ,  $p$ , and  $q$  are 0.

On the other hand, when a sensitizing dye is incorporated in a direct positive silver halide photographic emulsion, the sensitivity thereof may increase. However, in some instances the so-called "re-reversion" becomes

alkylthio group (such as a methylthio group or an ethylthio group), an arylthio group (such as a phenylthio group or a tolylthio group), an amino group, an alkylamino group or a substituted alkylamino group (such as a methylamino group, a dimethylamino group, a diethylamino group, a dodecylamino group, a cyclohexyl amino group, a  $\beta$ -hydroxyethylamino group, a di-beta-hydroxyethylamino group, or a beta-sulfoethylamino group), an arylamino group or a substituted arylamino group (such as an anilino group, an o-sulfoanilino group, a m-sulfoanilino group, a p-sulfoanilino group, an o-anisylamino group, a m-anisylamino group, a p-anisylamino group, an o-toluidino group, a m-toluidino group, a p-toluidino group, an o-carboxyanilino group, a m-carboxyanilino group, a p-carboxyanilino group, a hydroxyanilino group, a naphthylamino group, or a sulfonaphthylamino group), a heterocyclylamino group (such as a 2-benzothiazole-amino group or a 2-pyridylamino group), an aryl group (such as a phenyl group) or a mercapto group; and —A— represents a member of —A<sub>1</sub>— or —A<sub>2</sub>— as shown below.

—A<sub>1</sub>:



wherein  $M$  represents a hydrogen atom or a cation giving water solubility to the compound; and

—A<sub>2</sub>:



providing that when A is A<sub>2</sub>, at least one of said R<sub>1</sub>, R<sub>2</sub>, R<sub>3</sub> and R<sub>4</sub> is a substituent containing —SO<sub>3</sub>M, wherein M is the same as defined above.

## DETAILED DESCRIPTION OF THE INVENTION

Practical examples of the compounds represented by the general Formula I mentioned above are shown below:

Compound I-1:



wherein Y represents —CH— or —N—; R<sub>1</sub>, R<sub>2</sub>, R<sub>3</sub>, and R<sub>4</sub> each represents a hydrogen atom, a hydroxyl group, an alkoxy group, an aryloxy group (such as a phenoxy group, an o-toloxyl group, a p-sulfophenoxy group or a meta-naphthoxy group), a halogen atom (such as a chlorine atom or a bromine atom), a heterocyclic nucleus, an

5

### Compound I-2:



### Compound I-3:



### Compound I-4:



### Compound I-5:



### Compound I-6:



### Compound I-7:

6

5



### Compound I-8:

15



### 25 Compound I-9:

30



### Compound I-10:

40



50 Compound I-11:

55



The dyes represented by the general Formula I mentioned above are commercially available materials and well known.

65 The practical examples of the compounds represented by the general Formula II are shown below:

### Compound II-1:



### Compound II-2:



### Compound II-3:



### Compound II-4:



### Compound II-5:



### Compound II-6:



### Compound II-7:



### Compound II-8:



### Compound II-9:



### Compound II-10:



Compound II-11:



Compound II-12:



Compound II-13:



Compound II-14:



Compound II-15:



Compound II-16:



Compound II-17:



Compound II-18:



Compound II-19:



Compound II-20:



Compound II-21:



Compound II-22:



Compound II-23:



Compound II-24:



The compounds represented by general Formula II used in this invention are described in the specification of Japanese patent publication No. 10,773/68.

The dyes represented by the general Formula I used in this invention show no sensitizing effect in ordinary negative or positive photographic emulsions or have weak spectral sensitizing effect compared with cyanine sensitizing dyes or merocyanine sensitizing dyes. Therefore, it is astonishing to find that these dyes have an excellent sensitizing action to direct positive silver halide photographic emulsions.

65 The direct positive silver halide photographic emulsion sensitized by the dye of general Formula I is such that the photographic emulsion has a high sensitivity without reducing the maximum density ( $D_{max}$ ) and contrast by the addition of the dye. However, because the direct positive silver halide photographic emulsion sensitized by the dye of general Formula I exhibits "re-reversion" severely and the minimum density ( $D_{min}$ ) is high, such a photographic emulsion has not been employed practically.

As a compound for reducing the formation of the "re-reversion" and also the minimum density, a desensitizing compound such as pinakryptol yellow is known to be effective. However, when a desensitizing compound, such as pinakryptol yellow is incorporated in the direct positive silver halide photographic emulsion sensitized by the dye represented by the general Formula I, the  $D_{max}$  is scarcely reduced. However, such an attempt is accompanied with the defect that the reversal sensitivity is reduced together with the reduction of the formation of the "re-reversion" and the minimum density.

However, when the compound represented by the general Formula II is present together with the dye represented by the general Formula I in the direct positive silver halide emulsion according to the present invention, the maximum density is scarcely reduced and the formation of the "re-reversion" and the minimum density is also reduced. In addition, the reversal sensitivity does not reduce, but in some cases increases.

While the pinakryptol yellow, etc., exhibits a desensitizing property to ordinary negative or positive photographic emulsions, the compound represented by the general Formula II has almost no desensitizing property to such photographic emulsions and has no influence thereon. Thus, it is surprising that when the compound of the general Formula II is used together with the dye represented by the general Formula I, the formation of the "re-reversion" and the minimum density are reduced.

It is usually profitable to add to a silver halide photographic emulsion the dye represented by the general Formula I and the compound represented by the general Formula II as a solution of each. As the solvent for the dye represented by general Formula I, there is water, methanol, and ethanol. As the solvent for the compound represented by general Formula II, there is water, methanol and ethanol and as occasion demands, an alkali, such as sodium hydroxide, may be added to the solvent.

The effective amount of the dye shown by the general Formula II to be added to a direct positive silver halide photographic emulsion is 1-200 mg., and preferably 10-100 mg., per kilogram of the emulsion. The effective amount of the compound of general Formula II is 5-2,000 mg., and preferably 10-1,000 mg., per kilogram of the emulsion. The ratio of the compound of the general Formula I to the compound of the general Formula II is from 1/5 to 1/50 by weight.

In the silver halide emulsion employed in this invention, a silver salt such as silver chloride, silver bromide, silver chlorobromide, silver chloroiodide and silver chloroiodobromide may be used.

The emulsification and the physical ripening of the silver halide photographic emulsion used in this invention may be made in the manner conventionally employed for ordinary photographic emulsions, but a salt of the metal belonging to Group VIII of the Periodic Table, such as an iridium salt or rhodium salt may be added to the silver halide emulsion during the precipitation formation or during the physical ripening. The silver halide used in the present invention is fogged to the maximum density by light exposure or by a chemical fogging agent. The chemical fogging agent used for such purpose is required to fog the silver halide without imparting any deleterious effect to the silver halide emulsion, and usually thiourea dioxide, stannous chloride, formaldehyde or hydrazine is used. After the fogging operation is finished, the pH and  $P_{Ag}$  are controlled as the occasion demands.

A solution of the dye represented by the general Formula I is first added to a silver halide emulsion and then a solution of the compound represented by the general Formula II is added to the emulsion followed by stirring well. The silver halide emulsion is applied to a support.

The solution of the dye represented by the general Formula II may be added prior to the addition of the solution of the compound shown by the general Formula I, or a mixture of them may be added to the emulsion. Furthermore, these additives may be added to the silver halide emulsion during ripening after water washing. Moreover, ordinary additives, such as a wetting agent or a hardening agent, may be added to the silver halide emulsion.

As the support, there may be employed a glass sheet, a cellulose derivative film, a synthetic resin film, a baryta-coated paper, a waterproof paper, a laminated paper, etc.

#### BRIEF DESCRIPTION OF THE DRAWINGS

FIG. 1 is a graph showing a characteristic curve of a known emulsion.

FIG. 2 is a graph showing a characteristic curve of the emulsion according to this invention.

A better understanding of the present invention will be attained from the following example which is merely illustrative and not limitative of the present invention.

#### EXAMPLE 1

A silver chloroiodo-bromide emulsion (containing 1.3 mol percent iodine and 21.3 mol percent bromine) was fogged by formalin and the pH and  $P_{Ag}$  were adjusted to 5.6 and 6.7 respectively. The dye represented by the general Formula I was added to the emulsion followed by stirring and then the compound represented by the general Formula II was added thereto while the mixture was stirred sufficiently. The silver halide emulsion thus prepared was applied to a triacetyl cellulose film base. For the sake of comparison, a fogged silver halide photographic emulsion having the same composition as above to which, however, only the dye represented by the general Formula I had been added, was applied to the same kind of film base. After drying, each of the light-sensitive films thus prepared was exposed through a step wedge by means of a sensitometer and then developed in a developing solution having the following composition:

| Composition:               | G.  |
|----------------------------|-----|
| Metol                      | 4   |
| Hydroquinone               | 10  |
| Anhydrous sodium sulfite   | 60  |
| Anhydrous sodium carbonate | 2.5 |
| Water to make 1 liter.     |     |

The direct positive image obtained by the development was fixed by a fixing solution containing sodium thiosulfate, washed with water and dried. Thereafter, the optical density of the image was measured by means of a desensitometer. The results are shown in Table 1.

#### DETAILED DESCRIPTION OF THE DRAWINGS

The characteristic curves of a few samples in this example are shown in the graph of FIG. 2 and curves 2, 3 and 4 in FIG. 2 correspond to test numbers 9, 15 and 25, respectively. As is clear from these results, the reduction in sensitivity was observed in the sample containing pinakryptol yellow (pinakryptol yellow was added to the silver halide emulsion in place of the compound of the general Formula II, and the results are shown as Test No. 25 in Table 1 or the characteristic curve 4 in FIG. 2 for comparison).

Although the present invention has been sufficiently described in the foregoing specification and example included therein, it is readily apparent that various changes and modifications may be made without departing from the scope thereof.

TABLE I

| Test No. | Compound of Formula (I)<br>amount (mg./kg.-emulsion) | Compound of Formula (II)<br>amount (mg./kg.-emulsion) | White light<br>sensitivity<br>(Relative<br>value) | Maximum<br>(D <sub>max</sub> ) | Minimum<br>(D <sub>min</sub> ) |
|----------|------------------------------------------------------|-------------------------------------------------------|---------------------------------------------------|--------------------------------|--------------------------------|
| 1        | I-6 (27.5)                                           | II-1 (400)                                            | 100                                               | 23                             | 0.21                           |
| 2        | I-6 (27.5)                                           | II-1 (400)                                            | 100                                               | 22                             | 0.19                           |
| 3        | I-6 (27.5)                                           | II-1 (800)                                            | 95                                                | 22                             | 0.19                           |
| 4        | I-6 (27.5)                                           | II-2 (400)                                            | 98                                                | 22                             | 0.09                           |
| 5        | I-6 (27.5)                                           | II-2 (800)                                            | 95                                                | 22                             | 0.09                           |
| 6        | I-6 (27.5)                                           | II-4 (400)                                            | 110                                               | 23                             | 0.09                           |
| 7        | I-6 (27.5)                                           | II-4 (800)                                            | 100                                               | 22                             | 0.07                           |
| 8        | I-6 (27.5)                                           | II-8 (400)                                            | 115                                               | 23                             | 0.07                           |
| 9        | I-6 (27.5)                                           | II-8 (800)                                            | 112                                               | 23                             | 0.07                           |
| 10       | I-9 (30.0)                                           |                                                       | 100                                               | 23                             | 0.17                           |
| 11       | I-9 (30.0)                                           | II-3 (400)                                            | 100                                               | 23                             | 0.07                           |
| 12       | I-9 (30.0)                                           | II-5 (400)                                            | 103                                               | 22                             | 0.08                           |
| 13       | I-9 (30.0)                                           | II-6 (400)                                            | 124                                               | 23                             | 0.06                           |
| 14       | I-9 (30.0)                                           | II-7 (400)                                            | 124                                               | 22                             | 0.07                           |
| 15       | I-9 (30.0)                                           | II-8 (400)                                            | 148                                               | 23                             | 0.05                           |
| 16       | I-9 (30.0)                                           | II-9 (400)                                            | 105                                               | 22                             | 0.10                           |
| 17       | I-9 (30.0)                                           | II-10 (400)                                           | 100                                               | 22                             | 0.12                           |
| 18       | I-9 (30.0)                                           | II-11 (400)                                           | 120                                               | 23                             | 0.07                           |
| 19       | I-9 (30.0)                                           | II-12 (400)                                           | 112                                               | 23                             | 0.09                           |
| 20       | I-9 (30.0)                                           | II-13 (400)                                           | 100                                               | 23                             | 0.07                           |
| 21       | I-9 (30.0)                                           | II-14 (400)                                           | 98                                                | 22                             | 0.07                           |
| 22       | I-9 (30.0)                                           | II-15 (400)                                           | 105                                               | 23                             | 0.07                           |
| 23       | I-9 (30.0)                                           | II-16 (400)                                           | 128                                               | 23                             | 0.07                           |
| 24       | I-9 (30.0)                                           | II-17 (400)                                           | 105                                               | 22                             | 0.08                           |
| 25       | I-9 (30.0)                                           | Pinakryptol yellow (100)                              | 40                                                | 23                             | 0.05                           |
| 26       | I-8 (45.0)                                           |                                                       | 100                                               | 23                             | 0.15                           |
| 27       | I-8 (45.0)                                           | II-18 (800)                                           | 124                                               | 23                             | 0.08                           |
| 28       | I-8 (45.0)                                           | II-19 (800)                                           | 102                                               | 22                             | 0.10                           |
| 29       | I-8 (45.0)                                           | II-20 (800)                                           | 102                                               | 22                             | 0.08                           |
| 30       | I-8 (45.0)                                           | II-21 (800)                                           | 120                                               | 23                             | 0.08                           |
| 31       | I-8 (45.0)                                           | II-22 (800)                                           | 98                                                | 23                             | 0.08                           |
| 32       | I-8 (45.0)                                           | II-23 (800)                                           | 100                                               | 22                             | 0.12                           |
| 33       | I-8 (45.0)                                           | II-24 (800)                                           | 100                                               | 23                             | 0.09                           |

What we claim is:

1. A direct positive silver halide photographic emulsion having uniformly fogged silver halide grains containing a sensitizing effective amount of at least one dye represented by the general formula



wherein X<sub>1</sub>, X<sub>2</sub>, X<sub>3</sub>, X<sub>4</sub> and X<sub>5</sub> each represents a halogen atom; m, n, L, and p represent 0 or 1; q represents 0, 1, 2, 3 or 4; providing that when said m, n, L, p and q are 0, said X<sub>1</sub>, X<sub>2</sub>, X<sub>3</sub>, X<sub>4</sub> and X<sub>5</sub> each represents a hydrogen atom; and M represents a member selected from the group

consisting of a hydrogen atom, an alkali metal atom, NH<sub>4</sub>, and an alkaline earth metal; together with at least one compound represented by the general formula:



50 wherein Y represents a member selected from the group consisting of =CH— and =N—; R<sub>1</sub>, R<sub>2</sub>, R<sub>3</sub>, and R<sub>4</sub> each represents a member selected from the group consisting of a hydrogen atom, a hydroxyl group, an alkoxy group, an aryloxy group, a halogen atom, a heterocyclic nucleus, an alkylthio group, a heterocyclylthio group, an arylthio group, an amino group, an alkylamino group, a substituted alkylamino group, an arylamino group, a substituted arylamino group, a heterocyclamino group, an aryl group and a mercapto group; and —A— represents at least one member defined as A<sub>1</sub> and A<sub>2</sub>, said A<sub>1</sub> being a member selected from the group consisting of:



wherein M represents a member selected from the group consisting of a hydrogen atom and a cation giving water solubility to said compound; and said A<sub>2</sub> being a member selected from the group consisting of:



5



10

providing that when A is A<sub>2</sub>, at least one of said R<sub>1</sub>, R<sub>2</sub>, R<sub>3</sub> and R<sub>4</sub> is a substituent containing —SO<sub>3</sub>M, wherein M is the same as defined above, 20  
said compound of Formula II being present in an amount which will not decrease sensitivity.

2. The photographic emulsion of claim 1, wherein X<sub>1</sub>, X<sub>2</sub>, X<sub>3</sub> and X<sub>4</sub> in general Formula I represent a member selected from the group consisting of bromine and iodine, 25 and R<sub>1</sub>, R<sub>2</sub>, R<sub>3</sub> and R<sub>4</sub> in the general Formula II represent a member selected from the group consisting of an aryloxy group, an arylthio group, an arylamino group and a substituted arylamino group.

3. The photographic emulsion of claim 1, wherein the 30 dye of general Formula I is a member selected from the group consisting of:



35



40



45



50

55



75

and



claims 2 and 3 and the dye I of claim 15, wherein the photographic emulsion of claim 3, wherein said dye is a member selected from the group consisting of:

10 and



25 5. The photographic emulsion of claim 1, wherein the compound of the general Formula II is a member selected from the group consisting of:



21



22



23



and



6. The photographic emulsion of claim 5, wherein said compound is a member selected from the group consisting of:



and



7. The photographic emulsion of claim 1, wherein the amount of the dye represented by general Formula I is from 1 mg. to 200 mg. per kilogram of said silver halide emulsion.

8. The photographic emulsion of claim 1, wherein the amount of the compound represented by general Formula II is from 5 mg. to 2,000 mg. per kilogram of said silver halide emulsion.

9. The photographic emulsion of claim 1, wherein the ratio of the compound of general Formula I to the compound of general Formula II to be added to the silver halide emulsion is from 1/5 to 1/50 by weight ratio.

10. A silver halide photographic element comprising a support and a layer of the direct positive silver halide emulsion of claim 1.

11. The photographic emulsion of claim 7, wherein said dye is present in an amount of 10 mg. to 100 mg. per kilogram of said silver halide emulsion.

12. The photographic emulsion of claim 8, wherein said compound is present in an amount of from 10 mg. to 1,000 mg. per kilogram of said silver halide emulsion.

13. The photographic emulsion of claim 1, wherein the pH is 5.6.

14. The photographic emulsion of claim 1, wherein the  $p_{Ag}$  is 6.7.

#### References Cited

#### UNITED STATES PATENTS

20 3,537,858 11/1970 Wise \_\_\_\_\_ 96—107  
2,323,187 6/1943 Arens et al. \_\_\_\_\_ 96—64 X

NORMAN G. TORCHIN, Primary Examiner

W. H. LOUIE, Jr., Assistant examiner.

U.S. CL. X.R.

96—64, 107, 139